

# UNITED STATES PATENT OFFICE.

WILLIAM AUGUSTUS HALL, OF NEW YORK, N. Y.

## PROCESS FOR THE PRODUCTION OF SULFURETED HYDROGEN.

1,083,247.

Specification of Letters Patent. Patented Dec. 30, 1913.

No Drawing.

Application filed October 10, 1912. Serial No. 725,026.

To all whom it may concern:

Be it known that I, WILLIAM AUGUSTUS HALL, a citizen of the United States Republic, and resident of New York, N. Y., have invented a certain new and useful Improvement in Processes for the Production of Sulfureted Hydrogen, of which the following is a specification.

This invention relates to a new process for the production of sulfureted hydrogen from metallic sulfids, *e. g.*, iron pyrites and consists essentially in subjecting the sulfid, while agitating the same, to the combined action of a reducing flame (which decomposes it without producing any appreciable oxidation) and of steam or water vapor intended to furnish hydrogen. The combined and simultaneous action of the water vapor and of the reducing flame produces a much more active decomposition of the pyrites than that obtained by the flame alone. If no steam were present, the liberation of the sulfur would be slow and incomplete, whereas in presence of the steam, with which the sulfur of the pyrites can react, there is obtained a very active evolution of gas and a thorough decomposition of the pyrites. As the affinity of nascent hydrogen for sulfur at high temperature with the formation of  $H_2S$  is very great, the sulfur is easily and completely removed from the iron of the pyrites in a somewhat similar manner to its removal by oxidation with formation of  $SO_2$  when pyrites is burned in atmospheric oxygen.

In carrying this process into effect I proceed preferably as follows:—I heat the pyrites with a reducing flame obtained preferably from producer gas or so-called "gaz pauvre" and admit steam or water vapor at the same time as this gas, the pyrites being agitated throughout the operation. The two atoms of sulfur of the pyrites then combine with the hydrogen to furnish the sulfureted hydrogen. This result is to be attributed to the fact that the iron of the pyrites abandons practically all of its sulfur content in a reducing flame if it be furnished with a stable equivalent which will replace the sulfur and with which it can combine.

The process may easily be carried out in a continuous manner in a mechanical roasting furnace constructed as described in the specification of my co-pending application Serial No. 725,028, filed concurrently here-with.

It will be noted that a large amount of steam being admitted will produce a considerable depression of the temperature, in the reaction zone, which should be maintained by the combined action of the steam and reducing flame at a temperature somewhat below  $700^{\circ} C.$ , and at this temperature no material amount of sulfur (elemental) is distilled from the pyrites or other sulfid ore under treatment.

It is to be noted that with the furnace described in my application above referred to, very different conditions can be maintained than with a furnace of the blast or smelter type, since in my furnace, I maintain a layer of the ore, which is constantly being agitated, and the reducing flame plays upon the surface of the ore, there being no obstructions, and any desired amounts of air, gas and steam can be blown in, and fine ore can be used, and is even preferable to lump ore. In using a furnace of the smelter or blast furnace type, there is no agitation of the ore in the reaction zone, and the passage of the gaseous products of the reaction is always more or less restricted by the body of ore, (which practically excludes the use of fines) and the amount of air, gas and steam which can be introduced is determined by the amount of gases which can pass upwardly and out through the body of ore in the furnace.

The step of agitating the ore exercises two important functions in that it not only constantly exposes fresh surfaces to the action of the reducing flame, but it constantly intermingles the hot portions of the ore with the cooler portions thereof, and accordingly prevents local rises of temperature in those parts of the ore which are exposed to the direct action of the flame.

I make no claim to the carrying out of this process without a reducing flame, or in any except a reverberatory furnace, for the reasons that my process cannot be carried out without these two features being included.

The sulfureted hydrogen obtained by this process can be utilized for instance for the production of sulfur in accordance with the known formula:



The inventor is aware that it has been proposed to distil the sulfur of pyrites by means of highly superheated steam, but

processes based on this suggestion have met with no success because it was necessary to operate at a temperature higher than that to which steam could be economically superheated, and even at this very high temperature the reaction was very slow and never complete. The process covered by the invention differs radically from that mentioned above, being based on the fact that 10 the sulfur of the pyrites does not burn in a reducing flame, though the pyrites is decomposed, and when once it is decomposed in the presence of insufficient oxygen, its sulfur content in hot vaporous condition, will 15 combine easily with the hydrogen.

In carrying out the process of my present application, I admit a considerable amount of steam so that practically all the sulfur is driven out in the form of  $H_2S$  which 20 means that practically no sulfur is vaporized from the ore. Accordingly the temperature is maintained at a point somewhat below the point at which sulfur distils from the pyrites, namely about  $700^{\circ} C.$  or over. 25 The introduction of the steam in large amounts prevents the temperature from rising to a point above  $700^{\circ} C.$  By the use of less steam the temperature rises above  $700^{\circ} C.$  and a part of the sulfur will be distilled from the pyrites in the form of free 30 sulfur, this process being described and claimed in my copending application, Serial No. 725,024, filed concurrently herewith.

Having described my invention what I claim and desire to secure by Letters Patent 35 of the United States is:—

1. A process of producing  $H_2S$  from sulfid ore, which comprises agitating said ore, and subjecting the same to the combined action of a reducing flame and steam, the 40 steam being introduced in amount sufficient to maintain the ore at a temperature below that at which any material amount of free sulfur is vaporized.

2. A process of producing  $H_2S$  from sulfid ore, which comprises agitating a layer 45 of said ore, and subjecting the same to the action of a reducing flame blown directly upon the surface thereof, and to the simultaneous action of steam in large amount. 50

3. A process of producing  $H_2S$  from pyrites, which comprises agitating said pyrites, and subjecting the same to the combined action of a reducing flame and steam, the steam being introduced in amount sufficient 55 to maintain the pyrites at a temperature below that at which any material amount of free sulfur is vaporized.

In testimony whereof I have signed my name to this specification in the presence of 60 two subscribing witnesses.

WILLIAM AUGUSTUS HALL.

Witnesses:

HAROLD K. FAIRWEATHER,  
ALFRED T. BURBERRY.